

## UNITED STATES PATENT OFFICE

2,658,813

PROCESS OF SELECTIVELY CHLORIDIZING  
MANGANESE IN THE TREATMENT OF MA-  
TERIALS CONTAINING IRON AND MAN-  
GANESEIrving P. Whitehouse, South Euclid, and Marion  
Ernest Graham, Parma, Ohio, assignors, by  
mesne assignments, to Republic Steel Corpora-  
tion, Cleveland, Ohio, a corporation of New  
JerseyNo Drawing. Application October 5, 1951,  
Serial No. 250,032

7 Claims. (Cl. 23—87)

1

The present invention relates to a process of selectively chloridizing manganese in the treatment of materials containing iron and manganese. More particularly, the present invention relates to the treatment of materials, such as ores or semi-processed materials, which contain a preponderance of iron, usually in oxide form, and a relatively small amount of manganese, which may also be in oxide form, for the selective chloridizing of this material to produce a mixture of manganous chloride ( $MnCl_2$ ) and ferrous chloride ( $FeCl_2$ ), wherein the proportion of manganous chloride to ferrous chloride is at least about 1:1 and preferably about 4:1 or greater.

It has been known for some time that iron oxides, whether the iron be in the form of  $FeO$ ,  $Fe_2O_3$  or  $Fe_3O_4$ , may be reacted with hydrogen chloride (HCl) to form ferrous chloride. It is also known that manganese compounds, such as manganese oxides, may react with HCl to form manganous chloride ( $MnCl_2$ ). The prior art teaching generally is that the tendency of these two metallic oxides to be converted by reaction with HCl to the corresponding divalent chlorides is approximately equal. It is also known that if either iron or manganese is present in a material, alone or mixed together, they may be reduced from a higher valence form to a valence of two respectively by reduction with hydrogen. The combined reduction from a higher valence form to a valence of two and the conversion of the divalent metal to the chloride by reaction with HCl is known as to each of these metals individually. As far as is taught in the prior art, the tendency of the combined reduction and chloridizing reactions, as to each of these metals individually, is about equal. Based upon these known facts, it would reasonably be assumed by those skilled in the art, that if a material containing both these metals, in most or any of the forms in which these metals occur in nature, were exposed to a gas containing both hydrogen and HCl, the metals would be approximately equally converted to the respective chlorides. Thus, it would reasonably be expected that if an ore were treated in this way, and if the ore contained substantially more iron than manganese, as in the case of most naturally occurring ores of these two metals, the resulting chloride mixture, to the extent that it was formed, would contain the two metals in approximately the same proportion as that in which the metals were present in the original ore. This normally expected result is based upon known

2

activities of these two metals as aforesaid, both from the chemical and the thermodynamic points of view.

The present invention, however, is based upon an unexpected discovery, in that it is found that when a material, such as an ore or semi-processed material resulting from an ore, containing both iron and manganese, wherein the amount of iron present is substantially greater than the manganese present, is treated with a mixture of HCl and hydrogen, with or without other gases which are relatively inert insofar as the present process is concerned, the manganese is converted to manganous chloride to a far greater extent, at least at the first portion of the reaction, than the conversion of the iron to ferrous chloride. Thus, if such a solid material, as a natural ore, is maintained in a reaction zone at a temperature in a desired range, which has been found to be from about 300° F. to about 900° F., and more particularly and preferably from about 400° F. to about 800° F., and if the gas concentrations in the reaction zone are within certain desired limits as hereinafter set forth, the manganese will be converted to manganous chloride before too large a proportion of the iron is converted to ferrous chloride. This discovery may then be taken advantage of by stopping the process at the proper point to produce a soluble material, as a mixture of the chlorides of these two metals, which may be further treated in any desired way, some of which will be mentioned hereinafter, to produce a valuable mixture or alloy of iron and manganese, which is peculiarly and particularly useful, for example, as a source of manganese in the making of iron and steel. Thus such a material as the product of the present process may be treated to produce ferromanganese (an alloy containing about 80% manganese and 20% iron).

The present process may be summarized, therefore, as one in which a solid material of the type hereinabove described is treated in a reaction zone with a gas containing hydrogen and HCl, and at a temperature in the desired range as aforesaid, for a period terminating at a suitable time, so that the final product will contain at least 50% of the manganese initially present in the form of manganous chloride ( $MnCl_2$ ), and a relatively small proportion of the iron, not more than the amount of manganese as an outside limit, and preferably substantially less. This amount of manganese may be considered in respect to the iron either on a mol basis or on a weight basis, as both are substantially the same.

due to the similarity of the atomic weights of the iron and manganese. If the process were carried on under substantially the same conditions as herein contemplated, but for a too long time, it is recognized that more iron would be converted to ferrous chloride, so that the selectivity according to the present invention, would be effectively absent. Thus the present invention specifically contemplates terminating the operation of the process at a time when the chloridized material has a desired composition. This will be set forth in greater detail herein-after.

Turning now to the details of the present process, the first thing to consider is the composition and character of the raw material which may be treated according to the present process to produce results desired in accordance therewith. This material includes many naturally occurring ores as such. Among such ores which are contemplated for use in accordance with the present invention are:

(1) Georgia Ochre ore which is found, as the name implies, in various parts of the State of Georgia, having a typical analysis as follows:

|                                | Per cent |
|--------------------------------|----------|
| Total Fe                       | 42.40    |
| Ignition loss                  | 12.94    |
| SiO <sub>2</sub>               | 10.87    |
| Mn                             | 4.70     |
| Al <sub>2</sub> O <sub>3</sub> | 5.55     |
| P                              | 0.045    |
| CaO                            | 0.32     |
| MgO                            | 2.47     |
| BaSO <sub>4</sub>              | 4.50     |

(2) Red Aroostook ore which is found in Aroostook County, in the State of Maine, and having a typical analysis as follows:

|                  | Per cent |
|------------------|----------|
| Total Fe         | 31.91    |
| Ignition loss    | 9.51     |
| SiO <sub>2</sub> | 15.38    |
| Mn               | 12.09    |
| CaO              | 4.47     |

(3) Blue Aroostook ore, also found in Aroostook County, in the State of Maine, having a typical analysis as follows:

|                  | Per cent |
|------------------|----------|
| Total Fe         | 28.53    |
| Ignition loss    | 7.94     |
| SiO <sub>2</sub> | 14.39    |
| Mn               | 8.41     |
| CaO              | 3.65     |

It is also contemplated that various concentrates or semi-processed materials, including materials made from the ores aforesaid, may be similarly treated by the process of the present invention. It is further contemplated that materials resulting from other processes and which may contain more or less iron, usually in the form of one or more of its oxides, and manganese which may also be in the form of an oxide, such as MnO or MnO<sub>2</sub>, may be treated by the process of the present invention. The material may, therefore, be described generally as a solid material containing iron and manganese, in which the amount of iron present is substantially greater than the amount of manganese present. If the relative proportions of these materials were in the opposite ratio, the present process would generally be unnecessary, so that such materials are not contemplated for use as raw materials in accordance with this process. However, practically

all iron-manganese ores include a substantial preponderance of iron in respect to manganese and are, therefore, to be considered as suitable raw materials on which the present process may be practiced.

The next factor to be considered is the particle size required for the solid material aforesaid, for treatment according to the present process. Inasmuch as this is a gas-to-solid type reaction, relatively small particle size is usually desired. This will tend to increase the gas-to-solid contact and, therefore, will be desirable according to the present process. On the other hand, relatively large particle size, such as 8-mesh or larger, will introduce substantial difficulty, if not the complete impossibility, of contact between the gas and the material in the center of each large particle. As such, therefore, in the event that the original material to be treated is in relatively large particle size, it is desirable that it be suitably comminuted in any desired manner, to bring the particle size down to a point such that reasonably complete gas-to-solid contact is available. Some of the naturally occurring ores, such as Georgia Ochre, are normally in the form of fine particles. With this type of ore, little or no comminution is necessary. On the other hand, other types of ores, such as red or blue Aroostook ore are in the form of relatively large, hard lumps, which should first be comminuted before continuing with the steps of the present process, per se. It is usually preferred that the ore be of a particle size of 50-mesh and finer and preferably 100-mesh and finer. On the other hand, particle size is not absolutely critical, as it is essential only to obtain good gas-to-solid contact during the reaction.

The next factor to be considered is the type of apparatus in which the process is to be carried on. Inasmuch as the process involves a gas-to-solid contact reaction at a temperature which is elevated in respect to room temperature, any apparatus providing these conditions may be suitable for use. As many types of apparatus are now known wherein such conditions may be maintained, no one apparatus is particularly critical and none is illustrated in connection with the present application. The essential characteristics required for the apparatus to be used, are those which should provide good gas-to-solid contact, and which should provide for the maintenance of the desired temperatures for the reaction. In general, continuous types of apparatus are preferred in respect to intermittent or batch types, as the continuous types offer greater production in a given time. It is contemplated, for example, that suitable fluidized bed type apparatus is desirable for use, as this type of apparatus, which is now well known in the art, offers a maximum gas-to-solid contact, while permitting adequate temperature control. It is also contemplated that suitable rotary kiln type apparatus may be used; and it is noted in this connection that this type of apparatus was in fact used in connection with many of the examples of this process hereinafter set forth. In such apparatus a good gas-to-solid contact is afforded accompanied by a substantial degree of agitation, so that the gas can reach and react with substantially all the particles of the solid material. Other types of gas-to-solid contact apparatus, as will occur to those skilled in the art, preferably accompanied by agitation means, are also to be considered as feasible and operable in carrying out the present process. For the pur-

poses of the present application, any and all such apparatus is generally included in the term "reaction zone" into which this solid material is introduced and/or through which it is passed for the purposes of the present process.

The next factor to be considered is temperature. It has been found that the present process may be carried on advantageously in a temperature range having as its extreme limits from about 300° F. to about 900° F. It is noted that these temperature limits are both relatively low in respect to the temperature limits normally contemplated for the chloridizing of iron oxide-containing material with HCl where manganese is either absent or wherein the selective chloridizing of the manganese in respect to the iron is not particularly desired.

The reasons for choosing the present limits are that at temperatures as low as about 300° F., the hydrogen present in the gases as generally set forth hereinabove, does not seem to be particularly reactive to reduce the iron and manganese from a higher valence to a valence of two. Thus, for example, some of the iron may be chloridized to form ferric chloride ( $FeCl_3$ ) and the hydrogen present be relatively inactive to reduce this  $FeCl_3$  to  $FeCl_2$ . Inasmuch as the present process is intended to make ferrous chloride, to the extent that any iron is chloridized, as distinguished from ferric chloride, the temperature of 300° F. is selected as the effective and practical low temperature limit of the process.

The high temperature limit of 900° F. is chosen by reason of the desired selectivity of the reaction becoming progressively less as the temperature rises. Thus, at temperatures at or above about 900° F., the iron tends to chloridize almost as fast, if not faster, than the manganese. As such, at temperatures above about 900° F., selectivity, which is the principal feature of the present invention, is effectively absent. For this reason, therefore, about 900° F. is considered as the top limit for temperature in accordance with the present invention, and to attain the desired results thereof.

While the extreme limits have been chosen for the reasons aforesaid, a preferred range of temperature from about 400° F. to about 800° F. is set forth herein, these preferred limits being chosen based upon the same principles as set forth above as to the outside limits respectively, but with a purpose of keeping further away from the difficulties which cause the outside limits to be selected as aforesaid. Within this narrower preferred range, the desired results according to the present invention, are more certainly attained.

Another aspect of temperature is its general effect upon the rate of reaction. The present reaction, as in the case of many other chemical reactions, occurs more rapidly at higher temperatures. Thus, if it is desired to employ only a relatively short time of contact between the gas and the solid material, operations in the higher end or portion of the temperature range aforesaid are usually preferred. On the other hand, it must be kept in mind that the carrying on of the reaction is progressively more expensive as higher temperatures are used, due to the greater amount of heat required and the loss of such heat as sensible heat of the solid material at the completion of the reaction. The desired temperature may, therefore, be chosen finally based upon an economic balance between the speed of the reaction in the higher temperature ranges and the increased cost of maintaining the process

while operating in such higher temperature ranges.

The next factor to be considered is the gas composition. In general, the gas must contain both hydrogen and HCl. The requirements and effects of these two gases will now be separately considered.

As both the iron and the manganese may be in a valence state greater than a valence of two in the original material supplied to the process, some reduction of one or both these metals to a valence of two is usually necessary. Also, in the event that either of these metals were converted to a chloride having a valence greater than two, it is desired to convert such chloride to a divalent state and to reconstitute the remaining chlorine as HCl for the continuance of the reaction with unchloridized solid material. Thus, it is essential that some reducing agent, as hydrogen, be present. On the other hand, inasmuch as reduction is the only need for hydrogen, there need only be enough hydrogen to assure that there is always some hydrogen available to effect such reduction as may be required. In order to assure this, it is found that if the gases leaving the reaction zone contain at least some hydrogen, or in other words, contain at least a trace of hydrogen, then there is an assurance that there has been enough hydrogen to do everything that hydrogen can properly do. For this reason, therefore, the concentration of hydrogen in the incoming gases is not particularly important, but the presence of some hydrogen in the outgoing gases seems to be essential to assure the presence of hydrogen throughout the reaction. Excess of hydrogen does not appear to be at all harmful, as such excess hydrogen acts merely as an inert gas, insofar as the desired reaction is concerned.

As to the upper limit of hydrogen, it may be considered that there is always a possibility that hydrogen might react either with one or more of the oxides of iron, to reduce the iron from the oxide form to a metallic state or to reduce ferrous chloride to metallic iron. It is found, however, that either of these reactions will take place quite slowly until the uppermost range of temperature, in accordance with the present invention, is reached; and further, that the presence in the gases of some HCl will tend additionally to depress the rate of reduction of iron to the metallic state, irrespective of the iron compound which is to be reduced. On the other hand, it is practically impossible, in the temperature range according to the present invention, to reduce manganese to the elemental or metallic state with hydrogen, so that this possibility need not be seriously considered. As a practical matter, the presence of HCl in the concentrations normally used as herein set forth, will preclude all but a substantially negligible reduction of the iron to the metallic state except, perhaps in the temperature range above 800° F., and even at these temperatures, the rate of reduction of the iron is relatively slow in the presence of substantial amounts of HCl and is also retarded by water vapor. This possibility may, therefore, be effectively disregarded when operating according to the preferred range embodiment of the present process, even with the maximum amount of hydrogen permissible by differences between the amount of HCl present as hereinafter set forth and 100%. The only effective limit, therefore, upon the hydrogen concentration is that there should be sufficient hydrogen, so that the exit gases will contain at least a trace of hydrogen.

Examples of the hydrogen concentration in the gases as actually used in the practice of the process, will appear in the examples which follow.

The other essential ingredient in the gases, which are passed through the reaction zone, is HCl. This gas (HCl) is required to convert manganese and iron, which has been brought to a valence of two by the hydrogen, to MnCl<sub>2</sub> and FeCl<sub>2</sub> respectively. In view of the fact that the purpose of the process is primarily to convert the manganese present to MnCl<sub>2</sub>, there should be sufficient HCl present to do this. Thus, while the total amount of HCl to which the solid material is exposed while it is in the reaction zone, is not exactly critical, it is usual and is preferred to supply at least enough HCl into contact with the solid material, during the total period of contact between the solid material and the gases, to convert all the manganese present in the solid material to MnCl<sub>2</sub>. Thus, while the HCl concentration in the gases may be varied in different tests or in different operations during which the process is practiced, there must always be sufficient HCl to convert the amount of manganese to MnCl<sub>2</sub>, which it is desired to so convert, and preferably also enough to convert all the manganese present to MnCl<sub>2</sub>. On the other hand, it is not desired to convert iron to FeCl<sub>2</sub>, except to the extent that such conversion is unavoidable and is incidental to the desired conversion of manganese as aforesaid. For this reason, the iron content of the original raw material is not considered in determining how much HCl is to be used. Normally, it is quite usual to use more than enough HCl in respect to the stoichiometric amount required to convert all the manganese present to MnCl<sub>2</sub>, for example, one and one-half times as much as this stoichiometric amount. Under most circumstances, however, this ratio is probably to be considered as a high limit; as it is usually undesirable to use substantially more HCl than is necessary, as such excess HCl tends to increase the chloridization of the iron.

Thus far, the discussion has applied to the total amount of HCl in the gases in contact with any particular portion of the solid material during the passage of such portion through the reaction zone, or while such portion is in the reaction zone, as in the case of a "batch type operation" as to the solid type material. The concentration of HCl in the gases is not particularly critical. The essential feature is that during the time any portion of the solid material is in contact with the gases, sufficient HCl will be brought into contact therewith to effect desired results. This can be accomplished, therefore, by using a lower concentration and a longer time. However, in view of the fact that time is in most instances directly related to the economy of the process, it is usual to supply an HCl concentration such that the process may be completed to the extent desired in a reasonable time. Thus, while the concentration of HCl in the gases is not a critical factor, it is usual to use at least 6% HCl by volume in the gases, and preferably somewhat more, as illustrated by the examples which follow.

The gases passed through the reaction zone as aforesaid may also contain more or less inert gas, by which is meant gases which are inert, insofar as the present reaction is concerned, as well as those gases which are generally accepted as inert per se, such as nitrogen. It is desired, of course, that there be nothing in the gases

themselves which will interfere with the desired operation of the process. Therefore, the additional gases which may or may not be present, other than the essential gases, such as hydrogen and HCl, may be of any desired nature and may be present in any desired amount of concentration, as long as they do not interfere substantially with the operation of the process as herein set forth. Examples of gaseous mixtures including more or less inert gases will be given hereinafter.

The next point to be considered is the duration of the operation of the process, that is, the time of exposure of the solid material in the reaction zone to the gaseous mixture passing therethrough, while the temperature in such zone is suitably controlled and maintained as aforesaid. The process should be carried on for a time period sufficient to convert a desired and substantial amount of the manganese present to manganese chloride (MnCl<sub>2</sub>). For the purposes of the present application, this time period is selected as that in which at least 50% of the manganese present may be thus converted or chloridized. Normally, yields substantially greater than 50% of the manganese in the form of manganese chloride are desired, and are in fact attained as illustrated by many of the examples which follow. On the other hand, the process should not be continued for such a long period that iron is converted to the form of ferrous chloride to an undesired extent. In other words, it is essential that the process be not continued too long. This may be determined practically and with a very few experiments by the composition of the resulting solid material and may also be determined from an operational point of view by the composition of the exit gases as compared with the composition of the gases being supplied to the reaction zone, the rate of supply of such gases being known or predetermined. For example, it may be desired to make a product which will contain about 80% MnCl<sub>2</sub> and 20% FeCl<sub>2</sub> (considering only the chloridized material). Under such circumstances, when the amount of iron being chloridized tends to exceed about one part for every four parts of manganese chloridized, it is generally about time to stop the process, as a continuance of the process following this time will result in much more iron being chloridized than manganese. Examples of the amounts and proportions of iron and manganese chloridized will be given hereinafter, illustrating how the time for cessation of the process may be readily determined by those skilled in the art for any given set of conditions.

While no absolute theory can be given which will explain in detail or in full the desired results which are in fact attained by the present process, it is believed that when starting with a material, including a major portion of iron in some oxide form, and a relatively minor portion of manganese in some form, for example, an oxide form, the first things which happen are the simultaneous reduction of the two metals to a divalent state and then the conversion of some of the iron to a chloride form. Following this, it is believed that an interchange reaction occurs between ferrous chloride and MnO to give FeO plus MnCl<sub>2</sub>. The extent to which this interchange reaction occurs, as contrasted with the rate at which manganese oxide is chloridized by direct reaction with the gases, is not known. However, it is believed that the surprising re-

sults of the present process in the selective chloridizing of the manganese as compared with the iron, wherein as explained above, more or less equal results would be presumed in the absence of experimental proof, are due to the fact that this reaction occurs to some extent at least. With this exception, the reasons for the surprising results of the present invention are unknown. In any event, no particular theory is specifically relied upon in support of the patentability of the present invention; and the claims are to be considered accordingly.

Once the process proper has been completed in accordance with the present invention, it is desired usually to separate the chloridized manganese and iron from the remaining material. This can be effected by a leaching operation, due to the soluble character of the chlorides as contrasted with the insoluble character of the remainder of the original material, thus, the solid material resulting from the process, after it has been removed from the reaction zone and cooled to room temperature, may be leached with water to dissolve out the soluble chlorides, then the solution separated, as by filtration or decantation, from the insoluble material, and the soluble material recovered from the solution by evaporation.

Another way in which the manganese and iron chlorides may be removed from the remaining material is by vaporization that is, by heating the solid material up to a point where  $MnCl_2$  and  $FeCl_2$  will both vaporize. By condensing the resultant vapor, the chlorides may be recovered. By the use of a suitable gas, such as nitrogen or any other relatively inert gas, the temperature of vaporization of these chlorides may be brought down somewhat below the normal boiling points of these two chlorides as will be obvious to those skilled in the art.

Irrespective of the way the chlorides are separated from the remaining material as aforesaid, the metals may be recovered from the chlorides in any suitable way, forming per se no part of the present invention and which, therefore, are not specifically disclosed herein.

As illustrative of the practical operation of the process, the following examples may be given:

#### Example I

This example is given to illustrate the selective character of the present process as applied to different types of raw materials. For the purpose of this example, three different types of naturally occurring ores were used. In each test hereinafter given in this example, 150 gram samples of the ore was supplied to a rotary furnace three inches in inside diameter and five inches long. A gas composed of 80% hydrogen and 20% HCl was passed through this furnace for one hour, the rate of gas flow being such that during this time period, one and one-half times the stoichiometric amount of HCl was passed through the furnace, calculated in respect to the amount of HCl required to convert all the manganese present in the ore to  $MnCl_2$ . In each test the material in the furnace was maintained at about 600° F. In the first test hereinafter given a relatively easily chloridizable ore was used, so that the results stated show an adequate amount of chloridizing in accordance with the present invention; while in the other tests relatively difficultly chloridizable types of ores were used, so that the time period permitted was inadequate to effect the desired amount of chloridizing, accord-

ing to the present invention. However, even in the later tests, the selective character of the chloridizing is apparent.

A. Using Georgia Ochre ore of the composition given above and under the conditions stated, it was found that the resulting solid material contained 3.31% soluble manganese (as  $MnCl_2$ ), 0.95% insoluble manganese, 1.75% soluble iron (as  $FeCl_2$ ) and 43.2% insoluble iron. Thus 10 77.5% of the manganese was converted by the reaction to  $MnCl_2$ , while only 3.9% of the iron was converted to  $FeCl_2$ . In the soluble product, there was a ratio of manganese to iron of 1.9:1.

B. In this test Red Aroostook ore of the composition given above was used. Upon analysis of the solid product of the reaction, there was found 15 3.9% soluble manganese, 8.7% insoluble manganese, 0.4% soluble iron and 29.7% insoluble iron. Thus 31% of the manganese was converted to 20  $MnCl_2$ ; while only 1.3% of the iron was converted to  $FeCl_2$ . The ratio of the manganese to iron in the soluble final product was very high in this case, although this ratio is not considered as conclusive, as the process was not carried on for 25 a sufficient time for this type of raw material during this test. The selectivity, however, of the chloridizing is unquestionable.

C. In this test Blue Aroostook ore of the composition given above was used, giving a resulting 20 solid material containing 2.37% soluble manganese, 6.91% insoluble manganese, less than 0.1% soluble iron, and 30.1% insoluble iron. Thus, the manganese was 25.5% converted to  $MnCl_2$ , while less than 0.3% of the iron was converted to  $FeCl_2$ . 35 Again the test was carried on for too short a period of time to give proper results from the point of view of the present invention or to determine the eventual ratio of manganese to iron which would have been attained had the process 40 been carried on for a time period adequate for treating this type of ore.

#### Example II

The purpose of this example is to illustrate the 45 effect of varying temperatures on the reaction. In all tests in this example Red Aroostook ore of the composition given above was used.

A. In the first test illustrating the operation 50 of the process at a very low temperature, a 3.5 gram sample of the ore in a finely ground condition (all through 325 mesh) was exposed in a still bed to a gas containing, per minute of gas flow through the reaction chamber, 100 cc. HCl, 15 cc.  $H_2$  and 1520 cc.  $N_2$ . The temperature of the reaction chamber was maintained at about 300° F., and using a 360 minute test time period, the resulting product upon analysis, showed that 48.0% of the manganese present had been chloridized to  $MnCl_2$ , 2.8% of the iron had been 55 chloridized to  $FeCl_2$ , 7.8% of the iron had been chloridized to  $FeCl_3$ . The ratio of manganese to iron in the soluble portions of the solid product was 1.66:1. This test is considered to show that at this low temperature the reaction is quite selective, but due to the low temperature and to the presence of only a very small amount of hydrogen, a considerable amount of the iron was chloridized to ferric chloride, rather than ferrous chloride.

In a further test with conditions otherwise the same but with the temperature held at about 65 400° F. for 180 minutes, it was found that 72.5% of the manganese was chloridized to  $MnCl_2$  and 6.3% of the iron was chloridized to  $FeCl_2$ . In 70 this test there was no  $FeCl_3$  found in the final

## 11

product. Thus this test gave a soluble product having a ratio of manganese to iron of 4:47:1.

B. This test was carried on at a higher temperature within the preferred range, in this case with the rotary furnace which was described in connection with Example I, and using 150 mesh ore (Red Aroostook of the composition given above). The gas rates in this test (per minute) were 10 cc. H<sub>2</sub> and 50 cc. HCl. The gas was passed through the furnace for a total time of 162 minutes, during which time 110% of the stoichiometric amount of HCl (to convert all the manganese present to MnCl<sub>2</sub>) passed through the furnace.

In a first test under these conditions carried on at 600° F., 55.9% of the manganese was chloridized to MnCl<sub>2</sub> and 8.2% of the iron was chloridized to FeCl<sub>2</sub>, giving a soluble product having a ratio of manganese to iron of 2.66:1.

In a second test under these conditions, but with the temperature at 800° F., it was found that 79.4% of the manganese was chloridized to MnCl<sub>2</sub>, while 8.1% of the iron was chloridized to FeCl<sub>2</sub>, giving a manganese to iron ratio in the water-soluble product of 3.82:1.

C. A further test was carried on at the extreme high limit of temperature, 900° F.; in accordance with the present invention, this test being under the same still bed conditions described in respect to Example II (A) and using a 6.9 gram sample of the same Red Aroostook ore, the composition of which is given above. This sample was ground to all minus 100 mesh. The test was run for a period of 240 minutes, using 100 cc. of HCl and 400 cc. of H<sub>2</sub>, both per minute. The resulting material contained 89.4% of the Mn present as MnCl<sub>2</sub> and 58.6% of the Fe present as FeCl<sub>2</sub>, giving a ratio of manganese to iron in the soluble product of 0.61:1. This test is given to show that when the temperature is raised up to this high point, the tendency for iron to chloridize is so great in respect to the chloridization of the iron at lower temperatures, that the selectivity tends to go outside the desired range. Thus a temperature of about 900° F. may be considered as about the uppermost temperature limit at which the desired selectivity, in accordance with the present invention, is attained.

## Example III

This example is given to illustrate the effect of variations in the total amount of HCl used during the chloridizing reaction. In all tests in this example, Red Aroostook ore of the composition given above and having a grain size of minus 150 mesh was used in the same rotary furnace and generally under the conditions described in Example I. In all tests under this example, gas was passed through the furnace at the rate of 10 cc. of H<sub>2</sub> and 50 cc. of HCl, both per minute, and in all tests, the solid material was held at 600° F. The time of the reaction was varied in these several tests, so as to subject the solid material to differing total amounts of HCl.

A. In this test the stoichiometric amount of HCl required to convert all the manganese present to MnCl<sub>2</sub> was used. This took place in 147 minutes. The resulting solid material, upon analysis, showed that 50.7% of the manganese present had been converted to MnCl<sub>2</sub> and 3.5% of the iron present had been converted to FeCl<sub>2</sub>, giving a ratio of manganese to iron in the soluble product of 6.10:1.

B. In this test 110% of the stoichiometric amount of HCl was passed through the furnace

## 12

during a period of 162 minutes. The resulting product showed, upon analysis, that 55.9% of the manganese present had been converted to MnCl<sub>2</sub>, while 8.2% of the iron present had been converted to FeCl<sub>2</sub>, giving a ratio of manganese to iron in the soluble product of 2.66:1.

C. In this test 150% of the stoichiometric amount of HCl was used during a test period of 220 minutes. The final product, upon analysis, showed that 61.5% of the manganese present had been converted to MnCl<sub>2</sub> and 10.2% of the iron present had been converted to FeCl<sub>2</sub>, giving a ratio of manganese to iron in the soluble portion of the final product of 2.37:1.

## Example IV

This example is merely to bring out a comparison of prior tests, illustrating varying gas compositions (as to HCl) and includes a test in which there was a low HCl concentration in the gas present (see Example II-A) wherein only 100 cc. of HCl was present in a total of 1635 cc., or 6.13%. On the other hand, in Example III, substantially 83.3% of the total gas present was HCl.

There is further illustrated the effect of diluent gas in Example II-A, wherein nitrogen represented about 93% of the total gas present.

While there is herein disclosed in substantial detail all the essential elements of the present process and the ranges of equivalents where equivalents are reasonably contemplated, it is intended that the present invention shall be considered to include such reasonable equivalents as will occur to those skilled in the art from the foregoing disclosure.

What is claimed is:

1. The process of selectively chloridizing manganese in the treatment of material containing iron and manganese and in which the amount of iron present is substantially greater than the amount of manganese present, comprising the steps of introducing said material into a reaction zone, maintaining said material in said zone at a temperature in the range of about 300° F. to about 900° F., passing HCl into said zone to contact said material therein, supplying to said zone an amount of hydrogen sufficient so that the gases leaving said zone contain at least a trace of hydrogen, carrying on the steps aforesaid until at least about 50% of the manganese present has been converted to MnCl<sub>2</sub>, and discontinuing the process steps aforesaid when the ratio of manganese chloride to ferrous chloride produced is at least 1:1.

2. The process in accordance with claim 1, wherein the HCl concentration in said gases is at least about 6% by volume.

3. The process in accordance with claim 1, wherein said material is maintained in said zone at a temperature in the range of about 400° F. to about 800° F.

4. The process in accordance with claim 1, wherein said material is a naturally occurring ore, selected from the group consisting of Georgia Ochre, and Red and Blue Aroostook ores.

5. The process of selectively chloridizing manganese in the treatment of material containing iron and manganese and in which the amount of iron present is substantially greater than the amount of manganese present, comprising the steps of introducing said material into a reaction zone, maintaining said material in said zone at a temperature in the range of about 300° F. to

about 900° F., passing HCl into said zone to contact said material therein, supplying to said zone an amount of hydrogen sufficient so that the gases leaving said zone contain at least a trace of hydrogen, and discontinuing the process aforesaid when the conversion of iron to ferrous chloride tends to give a final product wherein the ratio of ferrous chloride to manganese chloride is greater than about 1:4.

6. The process of selectively chloridizing manganese in the treatment of material containing iron and manganese, and in which the amount of iron present is substantially greater than the amount of manganese present, comprising the steps of introducing said material into a reaction zone, maintaining said material in said zone at a temperature in the range of about 300° F. to about 900° F., passing HCl into said zone to contact said material therein until the amount of HCl passed through said zone is substantially 10 that amount required to convert all the manganese present in said material to MnCl<sub>2</sub>, supplying to said zone an amount of hydrogen suf-

5

ficient so that the gases leaving said zone contain at least a trace of hydrogen, and discontinuing the process steps aforesaid when the ratio of manganese chloride to ferrous chloride produced is at least 1:1.

7. The process according to claim 6, wherein said process is carried on with said material in said reaction zone at a temperature in the range of about 400° F. to about 800° F., and wherein said process is discontinued when the conversion of iron to FeCl<sub>2</sub> tends to produce more FeCl<sub>2</sub> in respect to the MnCl<sub>2</sub> produced than about 1:4 by weight.

IRVING P. WHITEHOUSE.  
MARION ERNEST GRAHAM.

## References Cited in the file of this patent

## UNITED STATES PATENTS

| Number    | Name        | Date          |
|-----------|-------------|---------------|
| 2,290,843 | Kinney      | July 21, 1942 |
| 2,425,995 | Christensen | Aug. 19, 1947 |